

1

3,496,620

**COMPOSITE ALUMINUM ARTICLE**

Wade Wolfe, Jr., Mount Carmel, Conn., assignor to Olin Mathieson Chemical Corporation, a corporation of Virginia  
No Drawing. Filed Nov. 7, 1966, Ser. No. 592,298  
Int. Cl. C22c 21/02, 21/04; B23n 3/00  
U.S. Cl. 29—183.5

7 Claims

**ABSTRACT OF THE DISCLOSURE**

A composite aluminous article having a core consisting essentially of from 0.2 to 2.8% magnesium, up to 1.0% silicon, up to 0.3% copper, up to 1.0% iron, from 0.10 to 1.5% manganese, up to 0.5% zinc, up to 0.5% chromium, said core clad with a dissimilar alloy consisting essentially of from 0.5 to 3.0% magnesium, up to 0.3% zinc, up to 0.4% silicon, up to 1.0% iron, up to 0.3% copper, up to 0.2% manganese, up to 0.3% chromium.

The present invention relates to composite metal articles. More particularly, the present invention resides in composite metal articles having an aluminous core and an aluminous cladding, said composites having improved corrosion resistance and improved mechanical properties.

Composite aluminum articles are widely known and have been used extensively in various applications. For example, composite aluminum articles are particularly well suited for uses involving exposure to supply waters because of their lightweight and good corrosion resistance.

It is known to provide a composite having a high strength aluminum alloy core, clad with either high purity aluminum or an aluminum alloy in order to provide a more corrosion resistant coating than the core alloy itself. For example, U.S. Patent 1,997,165 discloses composite aluminum articles having a cladding more electronegative than the core alloy in a sodium chloride-hydrogen peroxide solution in order to provide galvanic protection to the core material. It is a finding of this patent that various alloying additions to the cladding material, such as silver, gallium, bismuth, tin, zinc, etc. will provide an alloy having a more electronegative potential in a sodium chloride-hydrogen peroxide solution than most aluminum base alloy core materials and thereby improve the corrosion resisting properties of the composite.

A typical aluminum alloy composite based on this principle uses an aluminum plus zinc alloy cladding to protect the core from corrosion. One such clad composite has a 6061 aluminum alloy core and 7072 aluminum alloy cladding (throughout the specification, aluminum alloy numbers represent Aluminum Association designations). Aluminum alloy 6061 is a heat treatable wrought aluminum-magnesium-silicon alloy having nominal composition 1.0% magnesium, 0.6% silicon, 0.25% copper, and 0.25% chromium. Aluminum alloy 7072 has a nominal 1% zinc content in a commercial purity aluminum base. These composites do not give satisfactory service in many sections of the country. For example, the addition of zinc to aluminum decreases general corrosion resistance of aluminum in salt environments and in acidic conditions, such as industrial atmospheres. Accordingly, aluminum alloy 7072 is attacked by many atmospheres and becomes etched and disfigured by the accumulation of corrosion products. In addition, aluminum alloy 7072 is not particularly strong nor abrasion resistant and thereby detracts from the strength of many cores on which it is clad and provides a surface which is easily disfigured by abrasion.

Furthermore, alloy 7072 is sufficiently electronegative so that when tiny pits penetrate to the core-clad interface, the pits rapidly broaden by galvanic corrosion of 7072

2

and soon detract from the appearance of the clad surface. The zinc content of the clad alloy also presents a scrap recovery problem.

The foregoing disadvantages are true generally with cladding materials containing greater than 0.8% zinc. More noble core alloys, such as aluminum alloy 2024, are protected with relatively pure aluminum alloys. However, commercially available aluminum core materials containing magnesium as one of the major alloying elements are normally clad with high zinc containing alloys, such as 7072.

Accordingly, it is a principal object of the present invention to provide an improved composite alloy having an aluminous core and an aluminous cladding.

It is an additional object of the present invention to provide a composite material as aforesaid having improved corrosion resistance and improved mechanical properties.

It is an additional object of the present invention to provide an improved composite as aforesaid wherein the core material contains magnesium as one of the major alloying elements and the cladding has a low zinc content.

It is a still further object of the present invention to provide an improved composite as aforesaid which composite is strong and abrasion resistant and is not easily disfigured by abrasion.

A still further object of the present invention is to provide an improved composite as aforesaid which presents minimal scrap recovery problems.

Further objects and advantages of the present invention will appear hereinafter.

In accordance with the present invention it has now been found that the foregoing objects and advantages are readily obtained. The composite alloy of the present invention has a non-heat treatable core containing from 0.2 to 2.8% magnesium, from 0.10 to 1.5% manganese, up to 1.0% silicon, up to 0.3% copper, up to 1.0% iron, up to 0.5% zinc, up to 0.5% chromium, others 0.5% each, total 0.15% balance essentially aluminum, clad with a dissimilar alloy containing 0.5 to 3.0% magnesium, up to 0.3% zinc, up to 0.4% silicon, up to 1.0% iron, up to 0.3% copper, up to 0.2% manganese, up to 0.3% chromium, others 0.5% each, total 0.15%. The cladding should preferably contain more magnesium than the core and preferably at least 0.5% more magnesium than the core. In addition, the core should preferably contain more than the cladding of one or more of the following elements: copper, manganese and chromium.

The cladding material represents from 1.0 to 20% of the total thickness of the composite. The cladding may be on either one or preferably both sides of the core. Where the cladding is on both sides of the core it is preferred that each cladding represent from 1.0 to 10% of the total thickness of the composite per side.

It has been found in accordance with the present invention that the foregoing composite material readily overcomes the disadvantages of the art. The addition of magnesium to the cladding material provides stronger and more abrasion resistant composites than heretofore available. Furthermore, the aluminum-magnesium clad alloys of the present invention are more corrosion resistant than zinc containing claddings, such as aluminum alloy 7072. In the composites of the present invention the cladding galvanically protects the core but does not overprotect the core and waste the cladding. Hence, the cladding will have a longer life than zinc containing claddings, such as aluminum alloy 7072 and will maintain a better general appearance without unsightly broadening of pits through rapid and unnecessary galvanic corrosion of the cladding.

Furthermore, the aluminum-magnesium clad alloy of the present invention is totally acceptable for recycle, as

scrap, into production of those core alloys which also contain magnesium. Normally, composites having zinc containing aluminum alloy claddings, such as aluminum alloy 7072, suffer from the disadvantage that the zinc content of the cladding is incompatible with the production of many core alloys with which it is used.

The core material is any alloy falling within the foregoing compositional ranges. The core material contains magnesium in an amount from 0.2 to 2.8% and preferably from 0.8 to 1.1%. The core material is a non-heat treatable alloy and the cladding should preferably contain more magnesium than the core, with the cladding preferably containing greater than 0.5% magnesium than the core.

The core alloy may also contain the following ingredients in the following ranges: silicon up to 1.0%, preferably 0.15 to 0.7%, copper up to 0.3%, preferably 0.10 to 0.25%, iron up to 1.0% preferably 0.5 to 0.7%, manganese 0.1 to 1.5%, preferably 1.0 to 1.5%, zinc up to 0.5%, preferably up to 0.25%, chromium up to 0.5%, preferably 0.08 to 0.12%. In addition, it is desirable that these elements remain in solid solution in the aluminum alloy.

In addition, the core should preferably contain more than the cladding of one or more of the following elements: copper, manganese, and chromium in order to obtain a protective galvanic current between the cladding and the core alloys.

Typical core materials which may be employed include for example, aluminum 3004, 3105 and 5052.

The cladding material contains magnesium in an amount from 0.5 to 3.0%. In addition, the cladding may contain the following other materials. Zinc up to 0.3%, preferably up to 0.25%, silicon up to 0.4%, preferably up to 0.2%, iron up to 1.0%, preferably up to 0.5%, copper up to 0.3%, preferably up to 0.05%, manganese up to 0.2%, preferably up to 0.10%, chromium up to 0.3%.

Typical cladding materials include the following alloys: 5050, 5252, 5005 and so forth.

The method of forming the composite of the present invention is not particularly critical and any desired method for obtaining a metallurgically bonded composite may be employed, such as conventional casting, spraying or rolling techniques. For example, the core and cladding may be rolled together at from 800 to 1000° F. followed by rolling to finish gauge without an intermediate anneal at a temperature under 600° F.

The present invention and the improvements resulting therefrom will be more readily apparent from a consideration of the following illustrative examples.

#### EXAMPLE I

The following example describes the preparation of the typical composition of the present invention. Aluminum alloy 5050 was clad 5.8% on both sides of aluminum alloy 3004. The following steps were performed.

Step I—An ingot was cast of aluminum alloy 3004 of the size 16" x 45" x 85" and of the composition: silicon 0.22%, iron 0.62%, copper 0.14%, manganese 1.11%, magnesium 1.00%, zinc 0.03%, others less than 0.05%, total less than 0.15%.

Step II—The ingot was homogenized, and approximately 0.25" was scalped from each side.

Step III—A liner ingot was cast of aluminum alloy 5050 of the size 16" x 45" x 150" and of the composition: silicon 0.06%, iron 0.50%, copper 0.04%, manganese 0.02%, magnesium 1.53%, chromium 0.01%, zinc 0.03%, other less than 0.05% each, total less than 0.15%.

Step IV—The ingot of aluminum alloy 5050 was scalped, heated to 800° to 850° F., hot rolled to 1.00" gauge and sheared to provide two 1.00" x 43" x 83" slabs.

Step V—One liner slab of aluminum alloy 5050 was placed beneath the ingot of aluminum alloy 3004. An

additional liner slab of aluminum alloy 5050, as described above, was centered and placed upon the ingot. The total composite was heated for hot rolling at a temperature in range of 700° to 750° F.

Step VI—Metallurgical bonding of the 5050/3004/5050 composite was accomplished by hot rolling in a reversing mill which reduced the thickness to 0.702" gauge.

Step VII—While still hot, the composite was further reduced in a 3-stand mill to 0.2175" gauge. The hot mill sheet was slit to a 42" width, coiled and allowed to cool to room temperature.

Step VIII—The 5050/3004/5050 sheet was further reduced by cold rolling in three passes to 0.050" gauge.

Step IX—The cold rolled sheet was further slit into two coils together with the appropriate removal of scrap from the edges. One coil was 25.5" wide.

Step X—The 25.5" wide coil was flattened and sheared to provide flat sheets each 25.5" wide x 80" long x 0.050" gauge.

Step XI—Some of the sheets described in Step X were stabilized to the H-36 temper by a 2-hour soak at 300-325° F.

Step XII—The above stabilized sheets were then stretcher straightened.

Step XIII—One of the sheets from Step X was annealed to the O temper.

#### EXAMPLE II

The mechanical properties of the composite aluminum article, described above in Example I, are shown in the following table.

TABLE I

| Material       | Temper | 0.2% Offset Yield, p.s.i. | Ultimate, p.s.i. | Percent Elongation in 2" |
|----------------|--------|---------------------------|------------------|--------------------------|
| From Step X    | H-16   | 42,210                    | 43,450           | 2.8                      |
| From Step XII  | H-36   | 39,950                    | 41,980           | 5.8                      |
| From Step XIII | O      | 10,420                    | 25,130           | 20.6                     |

#### EXAMPLE III

Flat sheets of clad aluminum alloy 3004 (7072/3004/7072) were produced in a manner after Example I. The aluminum alloy 7072 cladding was of the composition: <0.10% silicon, <0.20% iron, <0.04% copper, <0.01% manganese, <0.02% magnesium, <0.01% chromium, 1.00% zinc and <0.030% titanium. The aluminum alloy 3004 core was of the composition: 0.21% silicon, 0.48% iron, 0.10% copper, 0.97% manganese, 0.91% magnesium, 0.003% chromium, 0.02% zinc and 0.015% titanium.

The mechanical properties of the above clad aluminum alloy 3004 in the 0.051 gauge are shown in the following table.

TABLE II

|                           |        |
|---------------------------|--------|
| Temper                    | H-36   |
| 0.2% offset yield, p.s.i. | 36,834 |
| Ultimate p.s.i.           | 39,818 |
| Percent elongation in 2"  | 6.3    |

Typical mechanical properties of clad aluminum alloy 3004 (7072/3004/7072) produced with this equipment are shown as the following average values from several lots of 0.500" gauge sheet.

TABLE III

|                           |        |
|---------------------------|--------|
| Temper                    | H-36   |
| 0.2% offset yield, p.s.i. | 37,500 |
| Ultimate p.s.i.           | 40,000 |
| Percent elongation in 2"  | 5.0    |

#### EXAMPLE IV

The composite aluminum article described in steps I through XII of Example I was sheared into 4" x 6" x 0.050" gauge panels.

Three of these panels were exposed for 1000 hours to neutral salt spray. This exposure was carried out by a procedure described in ASTM Designation B117-57T which requires a fog of 5% sodium chloride at 95 +2 to -3° F. It was found that the composite aluminum article was significantly more resistant to this environment than bare (unclad) aluminum alloy 3004 panels exposed during the same test.

Three additional panels of the composite aluminum article were exposed for 392 hours to acidified salt spray. This exposure was carried out by a procedure described in ASTM Designation B287-57R which requires a fog of 5+ sodium chloride solution, adjusted to a pH of 3.1 to 3.3, at a temperature of 95 +2 to -3° F. During this test it was found that aluminum alloy 5050 galvanically protected the underlying aluminum alloy 3004 core whereby pits were confined to a depth at or near the clad-core interface (the cladding thickness was 0.00289" on both sides). Considerable protection was afforded by the aluminum alloy 5050 clad compared to bare (unclad) aluminum alloy 3004 on which the average pit depth was found to be 9.6 mils and pits as deep as 18 mils were found during the same test.

#### EXAMPLE V

The above Example IV shows that aluminum alloy 5050 cladding will protect a core of aluminum alloy 3004 in accelerated test conditions. Galvanic protection was also found when equal areas of aluminum alloy 5050 and aluminum alloy 3004 were immersed in a 0.1 molar sodium chloride solution at temperatures of 25°-32° C., coupled outside the solution through suitable current measuring devices. The direction of current was such that aluminum alloy 5050 behaved electrochemically as an anode and aluminum alloy 3004 as a cathode without reversing direction of flow during 1.40 hours of measurement. The galvanic current was initially high and slowly decreased to a steady state value within about 120 hours. The total current expressed in coulombs, during 140 hours and the steady state current are shown in Table IV as Cell Number 3.

Table IV also shows that even higher protective currents can be obtained by increasing the copper content of the aluminum alloy 3004 cathode (Cell No. 4) or increasing the chromium content (Cell No. 5).

The galvanic currents found with other aluminum alloy clad-core combinations are shown as Cell Nos. 1, 2 and 6 in Table IV.

TABLE IV

| Cell No. | Electrode | Alloy | Percent |      |       |       |      |       |       |       | Total<br>Coulombs <sup>1</sup> | Steady<br>State<br>Galvanic<br>Current <sup>2</sup> |
|----------|-----------|-------|---------|------|-------|-------|------|-------|-------|-------|--------------------------------|-----------------------------------------------------|
|          |           |       | Si      | Fe   | Cu    | Mn    | Mg   | Cr    | Zn    | Ti    |                                |                                                     |
| 1        | Anode     | 5050  | 0.12    | 0.48 | <0.03 | <0.03 | 1.53 | <0.01 | <0.02 | 0.018 | 0.66                           | 1                                                   |
|          | Cathode   | 5052  | 0.10    | 0.28 | 0.05  | <0.03 | 2.30 | 0.19  | <0.03 | 0.01  |                                |                                                     |
| 2        | Anode     | 5252  | 0.05    | 0.02 | 0.01  | <0.01 | 2.35 | 0.02  | 0.07  | 0.008 | 1.83                           | 1.5                                                 |
|          | Cathode   | 5052  | 0.10    | 0.28 | 0.05  | <0.03 | 2.30 | 0.19  | <0.03 | 0.01  |                                |                                                     |
| 3        | Anode     | 5050  | 0.12    | 0.48 | <0.30 | <0.03 | 1.53 | <0.01 | <0.02 | 0.018 | 2.17                           | 2                                                   |
|          | Cathode   | 3004  | 0.25    | 0.78 | 0.10  | 1.19  | 1.19 | 0.24  | 0.018 | 0.018 |                                |                                                     |
| 4        | Anode     | 5050  | 0.12    | 0.48 | <0.03 | <0.03 | 1.53 | <0.01 | <0.02 | 0.018 | 2.03                           | 3                                                   |
|          | Cathode   | 3004  | 0.24    | 0.70 | 0.21  | 1.22  | 1.16 | 0.25  | 0.018 | 0.018 |                                |                                                     |
| 5        | Anode     | 5050  | 0.12    | 0.48 | <0.03 | <0.03 | 1.53 | <0.01 | <0.02 | 0.018 | 2.69                           | 3.5                                                 |
|          | Cathode   | 3004  | 0.26    | 0.78 | 0.10  | 1.23  | 1.08 | 0.123 | 0.24  | 0.008 |                                |                                                     |
| 6        | Anode     | 5252  | 0.05    | 0.02 | 0.01  | <0.01 | 2.35 | 0.02  | 0.07  | 0.008 | 5.16                           | 4.5                                                 |
|          | Cathode   | 3004  | 0.25    | 0.78 | 0.10  | 1.19  | 1.19 | 0.24  |       |       |                                |                                                     |

<sup>1</sup> Total coulombs during 140 hours.

<sup>2</sup> Galvanic current after 140 hours, micro-amperes per square inch.

This invention may be embodied in other forms or carried out in other ways without departing from the spirit or essential characteristics thereof. The present embodiment is therefore to be considered as in all respects illustrative and not restrictive, the scope of the invention being indicated by the appended claims, and all changes which come within the meaning and range of equivalency are intended to be embraced therein.

What is claimed is:

1. A composite aluminous article:

(A) having a core consisting essentially of from 0.2 to 2.8% magnesium, up to 1.0% silicon, up to 0.3%

copper, up to 1.0% iron, from 0.10 to 1.5% manganese, up to 0.5% zinc, up to 0.5% chromium, others each 0.05%, total 0.15%, balance essentially aluminum, said core being a non-heat treatable alloy;

(B) clad with a dissimilar alloy consisting essentially of from 0.5 to 3.0% magnesium, up to 0.3% zinc, up to 0.4% silicon, up to 1.0% iron, up to 0.3% copper, up to 0.2% manganese, up to 0.3% chromium, others each 0.05%, total 0.15%, balance essentially aluminum;

(C) wherein the cladding represents from 1.0 to 20% of the total thickness of the composite; and

(D) wherein said core contains more than said cladding of a material selected from the group consisting of copper, manganese and chromium.

2. A composite aluminous article:

(A) having a core consisting essentially of from 0.2 to 2.8% magnesium, up to 1.0% silicon, up to 0.3% copper, up to 1.0% iron, from 0.10 to 1.5% manganese, up to 0.5% zinc, up to 0.5% chromium, others each 0.05%, total 0.15%, balance essentially aluminum, said core being a non-heat treatable alloy;

(B) clad with a dissimilar alloy consisting essentially of from 0.5 to 3.0% magnesium, up to 0.3% zinc, up to 0.4% silicon, up to 1.0% iron, up to 0.3% copper, up to 0.2% manganese, up to 0.3% chromium, others each 0.05%, total 0.15%, balance essentially aluminum, said cladding containing more magnesium than said core;

(C) wherein the cladding represents from 1.0 to 20% of the total thickness of the composite; and

(D) wherein said core contains more than said cladding of a material selected from the group consisting of copper, manganese and chromium.

3. A composite according to claim 2 wherein the core is clad on both sides.

4. A composite according to claim 2 wherein said core contains from 0.8 to 1.1% magnesium, from 0.15 to 0.7% silicon, from 0.10 to 0.25% copper, from 0.5 to 0.7% iron, from 1.0 to 1.5% manganese, up to 0.25% zinc, and from 0.08 to 0.12% chromium.

5. A composite according to claim 2 wherein the cladding contains greater than 0.5% magnesium than the core.

6. A composite according to claim 2 wherein said alloying ingredients in said core are in solid solution.

7. A composite according to claim 2 wherein said cladding contains up to 0.25% zinc, up to 0.2% silicon,

up to 0.5% iron, up to 0.05% copper, and up to 0.10% manganese.

#### References Cited

#### UNITED STATES PATENTS

|           |         |          |          |
|-----------|---------|----------|----------|
| 1,805,448 | 5/1931  | Frary    | 29—197.5 |
| 1,997,166 | 4/1935  | Brown    | 29—197.5 |
| 2,726,436 | 12/1955 | Champion | 29—197.5 |

HYLAND BIZOT, Primary Examiner

U.S. Cl. X.R.